

Sept. 18, 1962

D. A. NEWMAN ET AL

3,054,692

NOVEL HECTOGRAPH METHODS

Filed Nov. 13, 1959

Fig. 1



Fig. 2



Fig. 3



Fig. 4



INVENTORS  
Douglas A. Newman  
Allan T. Schlotzhauer  
BY

Johnson and Kline  
ATTORNEYS

1

3,054,692

## NOVEL HECTOGRAPH METHODS

Douglas A. Newman, Glen Cove, and Allan T. Schlotz-  
hauer, Locust Valley, N.Y., assignors to Columbia Rib-  
bon and Carbon Manufacturing Co., Inc., Glen Cove,  
N.Y., a corporation of New York

Filed Nov. 13, 1959, Ser. No. 852,612  
6 Claims. (Cl. 117—17.5)

This invention relates to improvements in the thermo-  
graphic and xerographic methods of imaging hectograph  
master sheets, and more particularly to the use of novel  
heat-resistant hectograph transfer sheets in such methods.

It is known to prepare transfer sheets which carry  
a pressure-transferable layer of wax and color forming  
material and such sheets are the most common in use  
today. When a master sheet is placed over these sheets  
and pressure is applied, the said hectograph layer, cor-  
responding to the pressured areas, transfers to the master  
sheet. In the spirit duplication process, many copies can  
be made from the prepared master sheet.

However, these hectograph transfer sheets have cer-  
tain disadvantages. Of prime importance is the fact that  
a wax binder is not soluble in the fluids used to make  
spirit hectograph copies and further that the wax has a  
certain miscibility with modifying oils used in preparing  
the hectograph formulations. In other words, in a typical  
formula, approximately 10 to 15 parts of carnauba or  
other relatively high melting point vegetable waxes to-  
gether with approximately 10 to 15 parts lanolin and 10 to  
15 parts mineral oil are melted together. Naturally it is  
understood that other modifying agents such as castor oil,  
paraffin wax, butyl stearate, etc. can be included or re-  
place totally or in part the mineral oil and/or lanolin  
but the facts are that in general about one part of wax is  
used to two parts of modifying ingredients. In this event,  
the wax has miscibility with these materials so that the  
formula actually becomes more or less unified, all of  
which is not miscible with alcohol save perhaps those  
modifying agents such as butyl stearate or lard oil, castor  
oil, etc. that might be included, but in any case the wax  
base formula itself exhibits incompatibility with alcohol.

In using such a formula to prepare a hectograph ink,  
approximately one part of formula to two parts of dye  
are ground together and coated hot on the paper which  
on cooling solidifies, making a transfer film as originally  
described. In use, of course, the master having the hecto-  
graph formulation in image form is pressed against paper  
carrying a solubilizing fluid, principally alcohol, and as  
copies are produced the dye is leached out of the master.  
As the run continues, the ratio of dye to bonding agent  
reduces, particularly at the interface, until finally so  
little dye is taken off per copy that the copies are no  
longer acceptable. However, there is a great deal of  
dye remaining on the master that never is spent or dis-  
solved away because the wax forms a protective layer  
over the dye and only that amount of the color forming  
material which is present at or relatively near the surface  
of the wax image on the master sheet can be reached  
by the duplicating fluid and transferred to copy sheets.  
Thus the number of copies that can be derived is limited  
to the amount of dye that can be leached out in the  
above described manner. In short, the disadvantage  
with the known hectograph sheets is the fact that they  
contain only a limited amount of material which trans-  
fers to and stains the copy sheets. Thus a relatively large  
percentage of the image on the master sheet constitutes  
wax binding material which remains behind on the ex-  
pired master sheet and is wasted for imaging purposes.

Another serious disadvantage of the conventional hot  
melt wax hectograph transfer sheets is the fact that they

2

are meltable at temperatures in the range of 140° F. and  
above and therefore give rise to many problems when  
used in heat processes such as thermography and xero-  
graphy. Attempts to use these conventional hectograph  
transfer sheets in heat processes have failed since the wax  
coatings melt at the prevailing temperatures which range  
between 150°—450° F. and completely block off to the  
master sheet giving rise to a blurred master sheet and  
unrecognizable copies. In short, the transfer layer is  
transferred completely to the master sheet and no definite  
imaging occurs.

Therefore it is an object of the present invention to  
prepare hectograph transfer sheets which have none of  
the aforementioned disadvantages, and which provide for  
the preparation of sharper, more clear and more numerous  
copies through the spirit duplicating process than hereto-  
fore possible.

It is another object of the present invention to prepare  
spirit hectograph transfer sheets in which substantially all  
of the color forming material or dye is available for pro-  
ducing copies.

It is a further object of the present invention to prepare  
spirit hectograph transfer sheets in which the binding  
material does not interfere with the availability of the  
color forming material or dye for the imaging of copy  
sheets, and which is not wasted on the expired master  
sheet.

However it is the main object of the present invention  
to prepare hectograph transfer sheets which are heat stable  
and which do not melt at the temperatures required by  
the thermographic and xerographic processes.

These and other objects are accomplished in the manner  
disclosed hereinafter.

In the drawings:

FIGURE 1 is a diagrammatic cross-section, to an en-  
larged scale, of a master sheet and a hectograph transfer  
sheet having on the transfer layer xerographically-applied  
images superposed under the influence of heat but sepa-  
rated for purposes of illustration.

FIG. 2 shows the master sheet and hectograph transfer  
sheet of FIG. 1 after heating and separation.

FIG. 3 is a diagrammatic cross-section, to an enlarged  
scale, of a master sheet, a hectograph transfer sheet and  
an imaged original sheet superposed under the influence  
of infrared radiation in the thermographic process but  
separated for purposes of illustration.

FIG. 4 shows the master sheet and the hectograph transfer  
sheet of FIG. 1 after irradiation and separation.

According to the present invention, instead of wax as  
the binder, a cellulosic film-forming material such as ethyl  
cellulose is used which is at least partially soluble in the  
spirit duplicating fluids. Further, while the formulation  
contains oils, lanolin or other modifying agents in similar  
proportions to the wax base type, if they do become bonded  
with the ethyl cellulose they will transfer with the  
dye on copying since the ethyl cellulose is alcohol soluble.  
This situation also permits almost total exhaustion of the  
dye from the master, producing many more copies. It  
must be realized that formulations can be modified for  
copy brilliancy depending on the proportions of the non-  
volatile, non-miscible component to the bonding agent,  
that is to say, by changing either non-volatile component,  
cellulose or the dye proportions. Some dyes are much  
more soluble than others but in the last analysis the seal-  
ing properties of wax as against ethyl cellulose are such  
that the former seals while the latter more completely  
solvates thereby making available more dye from an im-  
pressed master sheet.

An equally important reason for the superior results  
obtained by plastic bonded type coatings is thought to be

that since the coating in the case of the cellulose bonded hectograph is applied with solvent and contains non-volatile, non-miscible materials, the cast film on drying is relatively porous having minute micellar structure, permitting alcohol to penetrate through the transferred image and in this way bringing about more complete solvation. Wax of course is insoluble in alcohol and prevents the penetration thereof.

When it is considered that each dye particle is surrounded by the vehicle in either case and when it is considered in the case of the cellulose film-forming material that the dye particles are surrounded by alcohol wettable resin, then it can be understood that dye solvation is more complete. Also the wettability of the dye by alcohol is improved over wax bonded formulas and exhaustion of the master takes place more completely.

While the above advantages (in respect to solvent resin bonded style of transfer coatings) are important from the standpoint of straight spirit hectograph duplication, the most important advantage from the standpoint of this invention is the heat resistance of the present transfer sheets.

There are at present two principal methods for accomplishing this which are applicable to forming hecto masters. One is xerography and the other, thermographic means involving infrared radiation.

In the first case, as illustrated by FIGS. 1 and 2 of the drawing, a xerographic image 15 may be formed on the face 11 of the solvent type of hectograph sheet 10 and that sheet together with a master 30 under sufficient pressure to hold the two firmly together subjected to heat 50 in which action the xerographic resin powder is fused in the imaged area so that the master and hectograph layer are "welded" together at said imaged areas. On separation after cooling, the dye layer is removed at said imaged areas and a master is thus prepared having the xerographic image 15 and a portion 35 of hectograph transfer layer adhered thereto.

The second consideration, that is to say thermographic means, as illustrated by FIGS. 3 and 4 of the drawing, the solvent type hectograph layer 11 may be cast on a more or less translucent base sheet 10 or a sheet at least which allows the penetration of infrared radiation. The said coated sheet together with a master 30 plus the copy sheet 20 having original images 21 thereon to be copied are fed through a thermographic machine having infrared radiation 50 in which act heat is developed in the image areas of the original, thereby causing a softening of the layer and "welding" the master in said areas to the hectograph sheet which on cooling and separation affords a mirror reverse facsimile image 31 on the master.

Now to further improve upon the "welding" of the master to the hectograph layer, it may be advisable to either film over the hectograph layer or apply a film to the master, said film having particular affinity for the master on the one hand or the hectograph layer on the other, as the case may be, when hot, thereby effecting a better, more complete transfer after cooling and separation. The whole point is that these solvent resin bonded type coatings, while they might soften with heat, do not flow out as does a wax coated sheet. Naturally it should be understood that a coating that becomes liquid under these temperatures is inoperable in the case of xerography to form a master as described because the whole hectograph mass would block off and adhere to the said master. Similarly, in the case of the thermographic method, the criticality would be much greater when flowable ink is used because of ambient temperature developed in the machine, whereas with a hectograph coating that does not become molten or fluid but merely softens, the criticality of the temperature factor is greatly reduced. Naturally, various modifications can be made in the composition of the resin bonded layer and/or undercoatings or supercoatings to fit an intended use, all of which will be well known in the art. The fact is that besides having a

better copying hectographic composition for regular work, an added advantage can be found in the application of the element to thermographic or xerographic duplicating methods.

5 The hectograph sheets of the present invention are prepared by coating a suitable foundation such as paper, cellulose acetate or Mylar, etc. with a coating of a cellulosic film-forming binder which is at least partially soluble in the conventional spirit duplicating fluids, non-volatile component which is not a solvent for the film-forming binder, hectograph dye material and filler, if desired. The coating may take place by dissolving the components in a volatile solvent, or by applying such coating in the form of an organosol or plastisol in a manner well known to the art. The preferred method, however, is the solvent application.

10 After application of the coating, the solvent is evaporated and there results the formation of a hectograph layer which does not melt at elevated temperatures but 15 becomes soft but not flowable at temperatures between 150°-450° F., which are the temperatures used in the thermographic and xerographic processes.

#### Example I

20 The following ingredients were thoroughly intermixed to a coatable consistency:

|                                                        | Parts by weight |
|--------------------------------------------------------|-----------------|
| Lard oil                                               | 8               |
| Oleic acid                                             | 8               |
| 30 Filler (if desired—may be graphite or carbon black) | 4               |
| Hectograph dye (Du Pont Spirit Black #3)               | 20              |
| Ethyl cellulose                                        | 5               |
| Solvent (toluol or the like)                           | 55              |
|                                                        | 100             |

35 The mixture was then spread evenly on a suitable base, such as paper, by suitable coating apparatus and allowed to cool and to set by evaporation of the solvent to form a smooth, pressure-transferable and heat-transferable hectograph coating having the properties described.

40 The prepared transfer sheet was then compared with a conventional hot melt wax hectograph sheet in the following manner: Two original sheets which were desired to be copied were placed face-up; then the novel 45 hectograph sheet of the present invention was placed face-up over the first original and the conventional hectograph sheet was placed face-up over the second original; next a suitable master sheet was placed over each of the transfer sheets, in contact with the hectograph layer, to form a pack. Each pack was then passed through a Thermo-Fax machine. The infrared radiation of the machine was focused on the master sheet and penetrated through to the original sheet where it was absorbed by the images on the original sheet and converted to heat in these areas. 55 The heat generated by the images causes the overlying transfer sheet to heat up over the imaged areas thereby bonding the master to said imaged areas.

55 Upon emergence from the machine, both packs were examined and tested. The pack carrying the conventional hectograph sheet was found quite inferior for many reasons. It appeared that the imaging layer of the conventional hectograph sheet had melted and become fluid at the existing temperatures and blocked off totally to the master sheet due to the overall ambient temperature of the thermographic machine and the lack of heat resistance of the transfer layer.

70 None of these defects was present in the pack containing the novel hectograph sheet of the present invention. It was found that the imaging layer of this sheet had not melted at the temperatures of the thermographic machine but merely became softened and adhesive over the image areas of the original sheet. The hectograph layer over these areas fused itself to the master sheet and transferred thereto in a substantially stenciling manner to give 75 a sharp, clear master sheet having minimal background

stains. Likewise it was found that the present transfer sheets permit for varying the density of the copies produced due to their heat resistance over a relatively wide temperature range. For instance, where denser copies and a longer running master sheet are desired, the speed at which the pack is run through the thermographic machine may be decreased thus allowing for increased heat formation in the imaged areas and a denser master sheet.

Each of the prepared master sheets was tested in a spirit duplicating machine and it was found that the novel sheets of the present invention resulted in cleaner, sharper and over 50% more numerous copies than the master sheet prepared from the conventional hectograph sheet.

*Example II*

|                                                   | Parts by weight |
|---------------------------------------------------|-----------------|
| Mineral oil                                       | 17.6            |
| Lanolin                                           | 3.2             |
| Hectograph dye material (Du Pont Spirit Black #3) | 19.2            |
| Ethyl cellulose                                   | 5               |
| Solvent (toluol or the like)                      | 55              |
|                                                   | 100.0           |

The above ingredients were mixed to a coatable consistency and coated on a suitable foundation as in Example I to form a hectograph transfer sheet.

This transfer sheet was then placed in face-to-face contact with a selenium plate carrying an electrostatic powdered image under sufficient pressure to keep the two elements in close contact. A corona discharge was applied, thereby reversing the polarity and upon removal of the hectograph sheet the powdered image adhered to the hectograph layer. The hectograph sheet bearing the powdered image was then placed in face-to-face contact with a master sheet to form a pack which was placed in a xerox oven at temperatures between 400°-450° F. and the powdered image fused and picked off the softened, non-fluid hectograph layer in the areas overlying the powdered images. Thus there was formed a master sheet, carrying a substantial amount of hectograph material in the electrostatic image areas, which may be used to prepare many sharp copies in the spirit process.

An attempt to employ conventional hot melt wax hectograph transfer sheets in this process failed due to the fact that the dye layer melted to a fluid state at the required temperatures and the fluid transferred to the master sheet throughout.

The proportions shown in the examples are not to be considered critical, the important factor being that the binder material is soluble in the spirit duplicating fluid. It has been found that amounts of binder as low as 2 or 3% based upon the total weight of the transfer composition may be used with excellent results, and that the amount of hectograph dye may be as high as 10 times the weight of binder used. The heat-resistance of the present transfer sheets appears to be due to the heat-resistance of the cellulosic resinous binder and the large amount of hectograph dye material employed.

No particular criticality exists with regard to the nature of the cellulosic binder so long as it is at least partly soluble and preferably completely soluble, in the spirit duplicating fluids employed. The preferred binders are the cellulose ethers, particularly ethyl cellulose which is very soluble in ethyl alcohol and mixtures of ethyl alcohol and water, which are the most common duplicating fluids. Other cellulosic binders which may be used include cellulose ethers such as methyl cellulose, carboxymethyl cellulose and others. It should be noted, however, that when the binder employed is water-soluble that the imaging material employed should be one which is not soluble in water. It is useful in some instances to overcoat the hectograph layer or coat the master sheet with a wax super-coating containing frangible, tacky material such as bees-

wax, Indopol and Vistanex to improve the attraction of the transfer layer from the master sheet.

It has been found that when the novel transfer sheets of the present invention are to be used in thermographic processes wherein the heat source is radiation such as infrared, then it is preferred that the master and transfer sheets be of such a nature as to allow the radiation to easily pass through. In this regard, transparent, translucent and transpicuous sheets are very satisfactory, such as clear plastic, frosted or crazed plastic, glassine paper, etc. Likewise the hectograph dye layer should be permeable to infrared radiation and should not contain any materials which absorb infrared radiation to any substantial degree. Suitable infrared-permeable dyes include rhodamine dyes, malachite green, safranine dyes and the like.

It has also been found that substantially colorless color-formers may be used in place of the colored dye on the transfer sheets. Such compounds are infrared-permeable and produce a bright color when brought in contact in the spirit process with complementary chemical reagents which are present on the treated copy sheets in the manner set forth in our copending application Serial No. 598,759, filed July 19, 1956, and now abandoned. For example, a compound such as gallic acid, tannic acid, rubanic acid, hematoxylin, sodium thiocyanate or any of the conventional color-formers as listed in the aforementioned application and in United States Patent No. 2,663,656 may be included in the ethyl cellulose layer in place of the hectograph dye. Copy sheets are prepared which are treated with complementary precipitant metal compounds such as those of iron, vanadium, copper, nickel, etc. as listed in the aforementioned application and patent. It is also possible to use substantially colorless unreacted dye components, one on the transfer sheet and the other on the copy sheets, which when brought together in the spirit process produce colored images.

One precaution must be observed, however, when using the aforementioned complementary color-forming compounds in thermographic processes of producing master sheets. When the transfer sheet and master sheet are heated together with the original to effect imaging of the master sheet, the temperature should be kept sufficiently low to prevent decomposition of the color-forming chemical and to compensate for the lower temperature the period of heating should be extended.

Variations and modifications may be made within the scope of the claims and portions of the improvements may be used without others.

50 We claim:

1. In the thermographic process of producing an imaged hectograph spirit master directly from original infrared radiation-absorbing images and a hectograph transfer sheet whereby the master, hectograph transfer sheet and the original images are superposed and infrared radiations are passed therethrough, the original images absorbing the same and converting them to heat, the improvement which comprises using as the hectograph transfer sheet one which does not absorb infrared radiation to any substantial degree and which carries a pressure-sensitive transfer layer which is based upon a cellulosic film-forming binder material containing a non-volatile component which is non-miscible with said binder material and which is selected from the group consisting of oleaginous and 55 pasty compositions, and a quantity of spirit-soluble imaging material, and the transfer layer softens but is non-fluid at temperatures between about 150° F. and 450° F., the temperature of the thermographic process.

2. The process of claim 1, wherein the hectograph transfer sheet comprises a flexible foundation having thereon a pressure-sensitive transfer layer comprising ethyl cellulose binder material which is at least partially soluble in the conventional spirit duplicating fluids, a mixture of lard oil and oleic acid and a quantity of spirit 60 soluble imaging material.

3. The process of claim 1, wherein the hectograph transfer sheet comprises a flexible foundation having thereon a pressure-sensitive transfer layer comprising ethyl cellulose binder material which is at least partially soluble in the conventional spirit duplicating fluids, a mixture of mineral oil and lanolin and a quantity of spirit-soluble imaging material.

4. In a xerographic imaging process of producing an imaged hectograph spirit master through the medium of a transfer sheet having a transfer layer thereon comprising hectograph imaging material, wherein an electrostatic image of electroscopic powder is formed on the surface of a xerographic plate, the electroscopic powder image is transferred so as to be positioned between the transfer layer on said transfer sheet and the surface of the master sheet and heat is applied to effect fusion of the electroscopic powder image and the underlying transfer layer comprising said hectograph imaging material to the master sheet whereby said imaged hectograph spirit master is formed upon separation of the sheets, the improvement which comprises using as the transfer layer on the transfer sheet one which is based upon a cellulosic film-forming binder material containing a non-volatile component which is non-miscible with said binder material and which is selected from the group consisting of oleaginous and pasty compositions, and a quantity of spirit-soluble imaging material, said transfer layer being non-fluid at temper-

atures between about 150° F. and 450° F., the temperature required for the heat transfer of the hectograph imaging material to the master sheet.

5. The process of claim 4, wherein the hectograph transfer sheet comprises a flexible foundation having thereon a pressure-sensitive transfer layer comprising ethyl cellulose binder material which is at least partially soluble in the conventional spirit duplicating fluids, a mixture of lard oil and oleic acid and a quantity of spirit-soluble imaging material.

6. The process of claim 4, wherein the hectograph transfer sheet comprises a flexible foundation having thereon a pressure-sensitive transfer layer comprising ethyl cellulose binder material which is at least partially soluble in the conventional spirit duplicating fluids, a mixture of mineral oil and lanolin and a quantity of spirit-soluble imaging material.

## References Cited in the file of this patent

## UNITED STATES PATENTS

|           |               |       |                |
|-----------|---------------|-------|----------------|
| 2,616,961 | Groak         | ----- | Nov. 4, 1952   |
| 2,808,777 | Roshkind      | ----- | Oct. 8, 1957   |
| 2,810,661 | Newman et al. | ----- | Oct. 22, 1957  |
| 2,930,106 | Wrotnowski    | ----- | Mar. 29, 1960  |
| 2,954,291 | Clark         | ----- | Sept. 27, 1960 |
| 2,954,311 | Vander Weel   | ----- | Sept. 27, 1960 |